# EUROPEAN PATENT SPECIFICATION

(11) **EP 2 298 944 B1**
(45) Date of publication and mention of the grant of the patent: **07.08.2013**
(21) Application number: 09171798.3
(22) Date of filing: 30.09.2009
(51) Int. Cl.: C22C 1/03, C22C 21/00, C22C 23/00

(54) **Method of manufacturing a magnesium-scandium master alloy and method of manufacturing an aluminum alloy containing scandium**
Herstellungsverfahren einer Magnesium-Scandium-Vorlegierung und Verfahren zur Herstellung einer Aluminiumlegierung, die Scandium enthält
Procédé de fabrication d'une alliage mère au magnésium-scandium, et procédé de fabrication d'une alliage d'aluminium contenant scandium

(30) Priority: 21.09.2009 KR 20090088959
(43) Date of publication of application: 23.03.2011
(73) Proprietor: Korean Institute of Industrial Technology, Cheonan-si Chungcheongnam-do 331-825 (KR)
(72) Inventor: Kim, Shea Kwang, 112-1903 Seoul (KR); Seo, Jung, Ho, 503-1305 Gyeongsangnam-do (KR); Kim, In Kyum, 104-1206 Chungcheongbuk-do (KR)
(74) Representative: Lippert, Stachow & Partner

(56) References cited:
- CN-C- 100 392 125
- RU-C1- 2 162 112
- RU-C1- 2 211 872
- RU-C1- 2 261 924
- US-A- 5 037 608
- US-A1- 2008 017 285
- WOO, KEE-DO ET AL: "Effects of grain size on high temperature deformation behavior of Al - 4Mg 0.4Sc alloy", MATERIALS LETTERS , 57(13-14), 1903-1909 CODEN: MLETDJ; ISSN: 0167-577X, 2003, XP002615558,

## Description

### BACKGROUND

### 1. Field

Example embodiments relate to a manufacturing method of a magnesium mother alloy and a method of manufacturing an aluminium alloy.

### 2. Description of the Related Art

Technologies of using scandium (Sc) as an additive in super-hard aluminum alloys (for example, 2000-series, 5000-series, 6000-series, 7000-series aluminum alloys, etc.) have recently been studied so as to improve alloy properties such as hardness, corrosion resistance and weldability. Aluminum alloys with Sc added may be used for military purposes (for example, reinforcement for combat vehicles, rifle bodies, etc.) requiring good weldability and fatigue resistance, or may be used for private purposes (for example, a high-speed train, parts for an electric train, etc.).

However, Sc is a rare earth material, and the amount of Sc existing on the earth is too small. Furthermore, there is a difficulty in separating Sc from a mineral, and thus Sc is very expensive.

Therefore, a method of adding scandium oxide (Sc₂O₃) into aluminum alloys is now being considered because Sc₂O₃ is relatively cheaper than Sc itself.

When, however, Sc₂O₃ is directly added into aluminum alloys, various alloy properties such as hardness, corrosion resistance and weldability are deteriorated due to oxides of Sc.

US 5 037 608 A discloses the addition of pellets of aluminum and Sc₂ O₃ into aluminum melts.

### SUMMARY

Embodiments are directed to a a manufacturing method of a magnesium mother alloy and a method of manufacturing an aluminum alloy, which substantially overcome one or more of the problems due to the limitations and disadvantages of the related art.

It is therefore a feature of an embodiment to provide a manufacturing method of a magnesium mother alloy with improved oxidation and ignition properties.

It is therefore a feature of another embodiment to provide a manufacturing method of an aluminum alloy with low cost, which is adapted for design purposes and does not deteriorate alloy properties such as hardness, corrosion resistance and weldability.

At least one of the above and other features and advantages may be realized by providing a magnesium mother alloy including: a plurality of magnesium grains; and scandium (Sc) dissolved in the magnesium grains.

The scandium may exist in an amount of about 0.0001 to about 30 parts by weight based on 100 parts by weight of magnesium.

At least one of the above and other features and advantages may be realized by providing a magnesium mother alloy including: a plurality of magnesium-aluminum grains having grain boundaries; and a scandium compound crystallized at the grain boundaries which are not inside but outside the magnesium-aluminum grains.

The scandium compound may include Al₂Sc, AlSc and Al₃Sc.

The scandium of the scandium compound may exist in an amount of about 0.0001 to about 30 parts by weight based on 100 parts by weight of the magnesium-aluminum

At least one of the above and other features and advantages may be realized by providing a method of manufacturing a magnesium mother alloy according to the appended claims.

In the forming of the magnesium melt, the magnesium may be pure magnesium or magnesium-aluminum.

An added amount of the scandium oxide may be about 0.0001 to about 30 parts by weight based on 100 parts by weight of pure magnesium or magnesium-aluminum

At least one of the above and other features and advantages may be realized by providing a metal alloy including: a plurality of metal grains having grain boundaries; and scandium dissolved in the metal grains, or a scandium compound crystallized at the grain boundaries which are not inside but outside the metal grains.

The metal may include one selected from consisting of AZ91 D, AM20, AM30, AM50, AM60, AZ31, AZ61, AZ80, AS41, AS31, AS21X, AE42, AE44, AX51, AX52, AJ50X, AJ52X, AJ62X, MR1153, MR1230, AM-HP2, Mg-Al, Mg-AI-Re, Mg-AI-Sn, Mg-Zn-Sn, Mg-Si, and Mg-Zn-Y.

The metal may include one selected from consisting of 1000-series, 2000-series, 3000-series, 4000-series, 5000-series, 6000-series, 7000-series and 8000-series wrought aluminum, and 100-series, 200-series, 300-series, 400-series, 500-series, and 700-series casting aluminum.

The scandium compound may include Al₂Sc, AlSc and Al₃Sc.

The scandium dissolved in the metal grains or the scandium of the scandium compound may exist in an amount of about 0.0001 to about 30 parts by weight based on 100 parts by weight of the metal.

At least one of the above and other features and advantages may be realized by providing a method of manufacturing an aluminum alloy according to the appended claims.

An added amount of the magnesium mother alloy containing scandium may be about 0.0001 to about 30 parts by weight based on 100 parts by weight of metal.

The magnesium mother alloy containing scandium may be manufactured by adding about 0.0001 to about 30 parts by weight of scandium oxide (Sc₂O₃) based on 100 parts by weight of pure magnesium.

The magnesium mother alloy containing scandium may be manufactured by adding about 0.0001 to about 30 parts by weight of scandium oxide (Sc₂O₃) based on 100 parts by weight of magnesium-aluminum.

The magnesium mother alloy containing scandium may include an alloy prepared by adding about 0.0001 to about 30 parts by weight of scandium oxide (Sc₂O₃) based on 100 parts by weight of pure magnesium, and an alloy prepared by adding about 0.0001 to about 30 parts by weight of scandium oxide (Sc₂O₃) based on 100 parts by weight of magnesium-aluminum.

The metal melt may be formed of one selected from consisting of AZ91D, AM20, AM30, AM50, AM60, AZ31, AZ61, AZ80, AS41, AS31, AS21 X, AE42, AE44, AX51, AX52, AJ50X, AJ52X, AJ62X, MR1153, MR1230, AM-HP2, Mg-Al, Mg-Al-Re, Mg-Al-Sn, Mg-Zn-Sn, Mg-Si, and Mg-Zn-Y

The metal melt may be formed of one selected from consisting of 1000-series, 2000-series, 3000-series, 4000-series, 5000-series, 6000-series, 7000-series and 8000-series wrought aluminum, and 100-series, 200-series, 300-series, 400-series, 500-series, and 700-series casting aluminum.

### BRIEF DESCRIPTION OF THE DRAWINGS

The above and other features and advantages will become more apparent to those of ordinary skill in the art by describing in detail exemplary embodiments with reference to the attached drawings, in which:

FIG. 1 is a flowchart illustrating a method of manufacturing a magnesium mother alloy according to an embodiment;

FIG. 2 is a micrograph illustrating a microstructure of a magnesium mother alloy in which scandium oxide is added into pure magnesium and Sc exists in a solid-solution state;

FIG. 3 is a micrograph illustrating a microstructure of a magnesium mother alloy in which scandium oxide is added to magnesium-aluminum and a scandium compound is crystallized;

FIG. 4 is a graph illustrating hardness comparison results between a pure magnesium and a magnesium mother alloy with scandium oxide added according to an embodiment;

FIG. 5 is a graph illustrating oxidation experimental results between a pure magnesium and a magnesium mother alloy with scandium oxide added according to an embodiment;

FIG. 6 is a graph illustrating ignition experimental results between a pure magnesium and a magnesium mother alloy with scandium oxide added according to an embodiment;

FIG. 7 is a graph illustrating hardness comparison results between a magnesium-aluminum alloy and a magnesium-aluminum alloy with scandium oxide added according to an embodiment; and

FIG. 8 is a flowchart illustrating a method of manufacturing a metal alloy according to an embodiment.

### DETAILED DESCRIPTION

Example embodiments will now be described more fully hereinafter with reference to the accompanying drawings; however, they may be embodied in different forms and should not be construed as limited to the embodiments set forth herein. Rather, the invention is defined by the appended claims.

FIG. 1 is a flowchart illustrating a method of manufacturing a magnesium mother alloy according to an embodiment.

The method of manufacturing the magnesium mother alloy includes forming a magnesium melt (S1), adding an additive (S2), stirring (S3), casting (S4), and cooling (S5).

In operation S1 of forming a magnesium melt, magnesium is put into a crucible and heated at a temperature ranging from about 600 °C to about 800 °C. Then, the magnesium in the crucible is molten to form a magnesium melt. Here, there is a difficulty in forming the magnesium melt when the temperature is less than 600 °C, whereas there is a danger that the magnesium melt is ignited when the temperature exceeds 800 °C.

Also, a small amount of a shield gas may be additionally provided to prevent the ignition of the magnesium melt. The shield gas may inhibit the ignition of the magnesium using SF₆, SO₂, CO₂, HFC-134a, Novec^{™}612, inert gas or an equivalent thereof, or a mixture gas thereof. However, in the embodiment, the shield gas may not necessarily used, and thus it may not be provided.

The magnesium used in operation S1 of forming the magnesium melt may be one selected from consisting of pure magnesium, magnesium-aluminum, and equivalents thereof.

In operation S2 of adding the additive, a powdered additive is added to the magnesium melt.

Here, the additive used in operation S2 of adding the additive may not be pure Sc of high price, but scandium oxide (Sc₂O₃) which is relatively cheap. The additive reduces the oxidation of a magnesium mother alloy, raises the ignition temperature, and remarkably reduces the required amount of the shield gas.

The additive used in operation S2 may be added in an amount of about 0.0001 to about 30 parts by weight based on 100 parts by weight of the magnesium mother alloy. When the amount of the additive is less than 0.0001 parts by weight, the effect (increase in hardness, decrease in oxidation, increase in ignition temperature and decrease in shield gas) resulting from the addition of the additive may be little. Also, when the amount of the additive exceeds 30 parts by weight, original magnesium properties or magnesium alloy properties may not appear.

The additive used in operation S2 may have a size ranging from about 0.1 µm to about 500 µm. It is difficult to manufacture an additive having a size of 0.1 µm or smaller actually, which requires high manufacturing cost. When the size of the additive exceeds about 500 µm, the additive may not react with the magnesium melt.

In stirring operation S3, the magnesium melt is stirred for about 1 to about 400 minutes.

When the stirring time is less than 1 minute, the additive is not sufficiently mixed with the magnesium melt. In contrast, when the stirring time is greater than 400 minutes, the stirring time of the magnesium melt is unnecessarily lengthened.

Here, the additive added into the magnesium melt does not exist in an oxide form. For example, when scandium oxide (Sc₂O₃) is added into the magnesium melt, it does not exist in the form of Sc₂O₃. That is, Sc₂O₃, after being reduced, reacts with elements in the magnesium melt so that Sc is dissolved in grains to exist in an alloy form, or crystallized to exist in a compound form.

Typically, it is expected that Sc₂O₃ is not reduced in the magnesium melt because Sc₂O₃ is thermodynamically more stable than magnesium. However, according to experiments conducted by the present inventors, it was found out that Sc₂O₃ is reduced in the magnesium melt. This reduction mechanism is not revealed yet, and therefore the present inventors continue to study in order to diagnose the reduction mechanism.

Substantially, when Sc₂O₃ is added into pure magnesium, Sc is dissolved in the pure magnesium. That is, Sc forms an alloy element with magnesium. In addition, when Sc₂O₃ is added into magnesium-aluminum, a Sc compound is crystallized at a grain boundary of the magnesium-aluminum. That is, Sc does not form an alloy element with magnesium but forms the Sc compound. Here, the Sc compound is in the form of Al₂Sc, AlSc or Al₃Sc typically.

Of course, the other elements (O₂) of the additives all float on the surface of the magnesium melt, and may be removed by manual or automatic equipment.

In casting operation S4, the magnesium melt is poured into a mold having a room temperature (e.g., about 25 °C) to about 400 °C, and then cast.

Here, the mold may be one selected from consisting of a metal type, a ceramic type, a graphite type and equivalents thereof. Also, a casting may be performed using gravity casting method, continuous casting method and equivalents thereof. However, the mold type and the casting method are not limited to the above.

In cooling operation S5, the mold is cooled down to a room temperature, and magnesium or magnesium-aluminum (e.g., ingot) is picked out of the mold.

Here, the magnesium mother alloy prepared through the above-described method, although will be explained below, may include a plurality of magnesium grains having grain boundaries therebetween, and Sc dissolved in the magnesium grains, or may include a scandium compound existing at the grain boundaries which are not inside but outside the magnesium grains.

FIG. 2 is a micrograph illustrating a microstructure of a magnesium mother alloy in which scandium oxide is added into pure magnesium and Sc exists in a solid-solution state. The microstructure shown in FIG. 2 is obtained by, for example, adding 0.5% scandium oxide into pure magnesium.

As shown in FIG. 2, a magnesium mother alloy 100 prepared according to an embodiment includes a plurality of magnesium grains 110, and scandium dissolved in the magnesium grains 110. Here, the scandium is not discriminated from the magnesium grains 110 substantially because scandium forms an alloy with magnesium.

Consequently, the hardness of the magnesium mother alloy manufactured by adding scandium oxide is improved compared to that of pure magnesium. In addition, since the scandium does not change the original composition of the magnesium mother alloy and does not disappear during a process of recycling the magnesium mother alloy, the reusability of magnesium mother alloy is considerably enhanced. That is, it is unnecessary to add scandium or scandium oxide again during the recycle of magnesium mother alloy.

Also, about 0.0001 to about 30 parts by weight of scandium oxide may be added based on 100 parts by weight of magnesium. The scandium oxide may have a size ranging from about 0.1 µm to about 500 µm. The meaning of such a numerical range has already been described above.

FIG. 3 is a micrograph illustrating a microstructure of a magnesium mother alloy in which scandium oxide is added to magnesium-aluminum and a scandium compound is crystallized. For example, the microstructure in FIG. 3 is obtained by adding 0.5% scandium oxide into magnesium-aluminum (Mg-3Al).

As shown in FIG. 3, a magnesium mother alloy 200 includes a plurality of magnesium-aluminum grains 210, and a scandium compound 211.

The plurality of magnesium-aluminum grains 210 have grain boundaries therebetween, and the scandium compound 211 exist at the grain boundaries which are not inside the grains 210 but outside the magnesium-aluminum grains 210. Here, the scandium compound 211 exists in the form of Al₂Sc, AlSc or Al₃Sc. That is, the scandium does not form an alloy with magnesium.

As such, the hardness of the magnesium mother alloy 200 is enhanced, which will be described below. Since the scandium does not change the original composition of the magnesium mother alloy and does not disappear during a process of recycling the magnesium mother alloy, the reusability of magnesium mother alloy is considerably enhanced. For example, it is unnecessary to add scandium or scandium oxide again during the recycle of magnesium mother alloy.

Also, about 0.0001 to about 30 parts by weight of the scandium compound 211 may be added based on 100 parts by weight of magnesium-aluminum. The scandium compound 211 may have a size ranging from about 0.1 µm to about 500 µm. The meaning of such a numerical range has been already described above.

The magnesium mother alloy may be used as one selected from consisting of an incombustible alloy, a wrought alloy, a creep alloy, a damping alloy, a degradable bio ally, and a powder metallurgy.

For example, the casting alloy may be formed by mixing AZ91 D, AM20, AM50, or AM60 with scandium oxide.

The wrought alloy may be formed by mixing AZ31, AM30, AZ61, or AZ80 with scandium oxide.

The creep alloy may be formed by mixing Mg-Al, or Mg-Al-Re with scandium oxide. Furthermore, the creep alloy may be formed by mixing Mg-Al-Sn or Mg-Zn-Sn with scandium oxide.

The damping alloy may be formed by mixing Mg, Mg-Si, or SiCp/Mg with scandium oxide.

The degradable bio alloy may be formed by mixing pure Mg with scandium oxide.

The powder metallurgy may be formed by mixing Mg-Zn-(Y) with scandium oxide.

Of course, in all the alloys, only scandium, which is obtained by removing O₂ from scandium oxide, is crystallized and present at grain boundaries, or the scandium exists in the grains in a solid-solution state finally.

FIG. 4 is a graph illustrating hardness comparison results between a pure magnesium and a magnesium mother alloy with scandium oxide added according to an embodiment. In FIG. 4, the X-axis represents a pure magnesium and a magnesium into which 0.5% scandium oxide is added, and the Y-axis represents hardness (HR).

As shown in FIG. 4, it can be observed that the hardness increases when scandium oxide is added during the manufacture of a magnesium mother alloy. That is, the hardness of the pure magnesium without scandium oxide is about HRF41, whereas the hardness of the magnesium mother alloy with scandium oxide added increases up to about HRF53.

FIG. 5 is a graph illustrating oxidation experimental results between a pure magnesium and a magnesium mother alloy with scandium oxide added according to an embodiment. In FIG. 5, the X-axis represents an elapse time (min.), and the Y-axis represents oxidation amount (%). A reference value of the Y-axis is set to 100.

As shown in FIG. 5, in the pure magnesium, it can be observed that the oxidation of the pure magnesium is accelerated with the lapse of time, and thus the value of the Y-axis increases gradually. However, in the magnesium mother alloy into which scandium oxide is added during manufacturing process, it can be observed that the oxidation does not increase even after the lapse of time. That is, the magnesium mother alloy is stable for various applications because it is not oxidized even after the lapse of time.

FIG. 6 is a graph illustrating ignition experimental results between a pure magnesium and a magnesium mother alloy with scandium oxide added according to an embodiment. In FIG. 6, the X-axis represents a pure magnesium and a magnesium into which 0.5% scandium oxide is added, and the Y-axis represents an ignition temperature (°C).

As illustrated in FIG. 6, it can be observed that the ignition temperature of the magnesium mother alloy with scandium oxide added is increased. That is, the ignition temperature of the pure magnesium without scandium oxide is about 600 °C, whereas the ignition temperature of the magnesium mother alloy with scandium oxide added increases up to about 700 °C.

FIG. 7 is a graph illustrating hardness comparison results between a magnesium-aluminum alloy and a magnesium-aluminum alloy with scandium oxide added according to an example embodiment. In FIG. 7, the X-axis represents a magnesium-aluminum alloy and a magnesium-aluminum alloy into which 0.5% scandium oxide is added, and the Y-axis represents hardness (HR).

As shown in FIG. 7, it can be observed that the hardness increases when scandium oxide is added during the manufacture of a magnesium-aluminum alloy. That is, the hardness of the magnesium-aluminum alloy without scandium oxide is about HRF50, whereas the hardness of the magnesium-aluminum alloy with scandium oxide added increases up to HRF68.

FIG. 8 is a flowchart illustrating a method of manufacturing a aluminum alloy according to an embodiment.

The method of manufacturing the metal alloy includes forming a aluminum melt (S11), adding a magnesium mother alloy containing scandium (S12), stirring (S13), casting (S14), and cooling (S15), as described in the appended claims.

Also, the aluminum may be a metal alloy selected from consisting of 1000-series, 2000-series, 3000-series, 4000-series, 5000-series, 6000-series, 7000-series and 8000-series wrought aluminum, and 100-series, 200-series, 300-series, 400-series, 500-series, and 700-series casting aluminum.

Herebelow, the aluminum alloys will be more specifically described. Various kinds of aluminum alloys have been developed for their use, and most of countries currently classify the kinds of aluminum alloys according to the standard stipulated by the Aluminum Association of America. Main alloy elements for each of alloy series are listed in Table 1 below in which a serial number is only shown in units of thousand. In case of improving each of the alloy series by adding other elements, an alloy name is designated by subdividing four digits number more specifically.

**[Table 1] Classification of aluminum according to alloy series**

| Alloy Series | Main alloy elements |
|---|---|
| 1000-series Al | Pure Al |
| 2000-series Al | Al-Cu-(Mg)-based Al alloy |
| 3000-series Al | Al-Mn-based Al alloy |
| 4000-series Al | Al-Si-based Al alloy |
| 5000-series Al | Al-Mg-based Al alloy |
| 6000-series Al | Al-Mg-Si-based Al alloy |
| 7000-series Al | Al-Zn-Mg-(Cu)-based Al alloy |
| 8000-series Al | Others |

The first number denotes an alloy series representing main alloy elements, and the second number denotes whether a basic alloy is improved or not. That is, the second number of 0 represents a basic alloy, and the second number of 1 to 9 represents alloys improved from the basic alloy. Further, when a new alloy is developed, the second number is indicated by a capital letter N. For example, 2xxx represents a basic alloy of Al-Cu series aluminum, 21xx∼29xx represents alloys obtained by improving an Al-Cu basic alloy, and 2Nxx represents a newly developed alloy which is not stipulated in the standard of the Aluminum Association of America. The third and fourth numbers represent the purity of a pure aluminum or an alloy name of an aluminum alloy that Alcoa Inc. has used in the past. For example, in case of pure aluminum, 1080 indicates that the content of aluminum is 99.80% or higher, and 1100 indicates that the content of aluminum is 99.00% or higher.

Main compositions of wrought alloys are listed in Table 2 below. Properties of each alloy may significantly differ according to composition metals and their amounts, and working process.

The main composition of the aluminum alloy is listed in Table 2 below.

**[Table 2] Main composition of aluminum alloy**

| Grade | Added metal(element symbol), Unit: % | | | | | | | Use |
|---|---|---|---|---|---|---|---|---|
| | Si | Cu | Mn | **Mg** | Cr | Zn | others | |
| 1100 | | 0.12 | | | | | Si 1%, Abundant Metal | foils, cooking utensils |
| 1350 | | | | | | | About others | 0.5% Conductive material |
| 2008 | 0.7 | 0.9 | | **0.4** | | | | Metal plates for vehicles |
| 2014 | 0.8 | 4.4 | 0.8 | **0.5** | | | | Exterior of aircraft, truck frame |
| 2024 | | 4.4 | 0.6 | **1.5** | | | | Exterior of aircraft, truck wheel |
| 2036 | | 2.6 | 0.25 | **0.45** | | | | Metal plates for vehicles |
| 2090 | | 2.7 | | | | | Li 2.2, Zr 0.12 | Metal for aircraft |
| 2091 | | 2.2 | | **1.5** | | | Li 2.0, Zr 0.12 | Metal for aircraft |
| 2219 | | 6.3 | 0.3 | | | | V 0.1, Zr 0.18, Ti 0.06 | Metal for spacecraft, weldable |
| 2519 | | 5.9 | 0.3 | **0.2** | | | V 0.1, Zr 0.18 | Military equipment, metal for spacecraft, weldable |
| 3003 | | 0.12 | 1.1 | | | | | General use, cooking utensils |
| 3004 | | | 1.1 | **1.0** | | | | General use, metal can |
| 3105 | | | 0.6 | **0.5** | | | | Building materials |
| 5052 | | | | **2.5** | 0.25 | | | General use |
| 5083 | | | 0.7 | **4.4** | 0.15 | | | Heat-/Pressure-resistant vessels |
| 5182 | | | 0.35 | **4.5** | | | | Metal can, metal for vehicles |
| 5252 | | | | **2.5** | | | | For vehicle bodies |
| 6009 | 0.8 | 0.33 | 0.33 | **0.5** | | | | Metal plates for vehicles |
| 6010 | 1.0 | 0.33 | 0.33 | **0.8** | | | | Metal plates for vehicles |
| 6013 | 0.8 | 0.8 | 0.5 | **1.0** | | | | Metal for spacecraft |
| 6061 | 0.6 | 0.25 | | **1.0** | 0.20 | | | General use |
| 6063 | 0.4 | | | **0.7** | | | | General use, injection molding |
| 6201 | 0.7 | | | **0.8** | | | | Conductive material |
| 7005 | | | 0.45 | **1.4** | 0.13 | 4.5 | Zr 0.14 | Truck body, train |
| 7075 | | 1.6 | | **2.5** | 0.25 | 5.6 | | Metal for aircraft |
| 7150 | | 2.2 | | **2.3** | | 6.4 | Zr 0.12 | Metal for spacecraft |
| 8090 | | 1.3 | | **0.9** | | | Li 2.4, Zr 0.12 | Metal for spacecraft |

In operation S12 of adding the magnesium mother alloy, a magnesium mother alloy containing Sc is added to the aluminum melt.

The magnesium mother alloy used in operation S12 is manufactured in accordance with claims 1-3.

In this way, according to an exemplary embodiment, magnesium or magnesium-aluminum alloy containing scandium that is prepared at low cost is added into a metal melt, thus making it possible to solve several problems occurring when scandium oxide is directly put into the metal melt. For example, the direct addition of scandium oxide (Sc₂O₃) into aluminum causes the quality of an alloy to be deteriorated due to oxides, however, the quality of an alloy is not deteriorated by adding magnesium or magnesium-aluminum alloy containing scandium according to the embodiment. More specifically, alloy properties such as hardness, corrosion resistance and weldability are deteriorated when scandium oxide (Sc₂O₃) is directly added into aluminum, however, alloy properties such as hardness, corrosion resistance and weldability in the metal alloy according to the embodiment are maintained without a change when magnesium or magnesium-aluminum already containing scandium is added into aluminum.

For instance, 5000-series metal alloys are strong, easy to be molded, and highly resistant to corrosion, in comparison with 3000-series metal alloys. Furthermore, 5000-series metal alloys are weldable. In particular, the 5182 alloy may be used for a cover of an aluminum can. In addition, 5005 and 5083 alloys, and 5052, 5056, 5086 and varieties thereof may widely be used for electric facilities, various cooking utensils, metal plate, pressure-resistant vessels, transmission towers of radio wave, welding structures, boats, reservoirs for chemicals, etc. Insect nets, nails, and fasteners may be made of 5000-series alloys. When magnesium or magnesium-aluminum alloy already containing scandium is added into such 5000-series metal alloys having the above properties, it is possible to obtain an aluminum alloy with good hardness, corrosion resistance and weldability at low cost.

The additive used in operation S12 of adding the magnesium mother alloy may be added in an amount of about 0.0001 to about 30 parts by weight based on 100 parts by weight of the metal. When the amount of the additive is less than 0.0001 parts by weight, the effect (hardness, corrosion resistance, and weldability) resulting from the addition of magnesium may be little. Also, when the amount of the additive exceeds 30 parts by weight, original metal properties may not appear.

Furthermore, the additive used in operation S12 of adding the magnesium mother alloy may have a size ranging from about 0.1 µm to about 500 µm. It is difficult to manufacture an additive having a size of 0.1 µm or smaller actually, leading to high manufacturing cost. When the size of the additive exceeds 500 µm, the magnesium may not react with the metal melt.

Likewise, the additive used in operation S12 of adding the magnesium-aluminum may be added in an amount of about 0.0001 to about 30 parts by weight based on 100 parts by weight of the metal alloy. When the amount of the additive is less than 0.0001 parts by weight, the effect (hardness, corrosion resistance, and weldability) resulting from the addition of magnesium may be little. Also, when the amount of the additive exceeds 30 parts by weight, original metal properties may not appear.

Furthermore, the additive used in operation S12 of adding the magnesium-aluminum may have a size ranging from about 0.1 µm to about 500 µm. It is difficult to manufacture an additive having a size of 0.1 µm or smaller actually, leading to high manufacturing cost. When the size of the additive exceeds 500 µm, the of adding the magnesium-aluminum may not react with the metal melt.

In stirring operation S13, the metal melt is stirred for about 1 to about 400 minutes.

When the stirring time is less than 1 minute, the additive is not sufficiently mixed with the metal melt. In contrast, when the stirring time is greater than 400 minutes, the stirring time of the metal melt is unnecessarily lengthened.

As the metal melt is an aluminum melt, scandium contained in the magnesium added into the aluminum melt exists in the form of Al₂Sc, AlSc or Al₃Sc due to the high affinity between Sc and Al.

In stirring operation S13, Al₂Sc, AlSc or Al₃Sc does not exist in metal grains, but exists outside the metal grains, i.e., at grain boundaries, in the form of an intermetallic compound. That is, the metallic compound of Al₂Sc, AlSc or Al₃Sc is formed in stirring operation S13.

In casting operation S14, the metal melt is poured into a mold at a room temperature (e.g., about 25 °C) to about 400 °C, and then cast.

Here, the mold may be one selected from consisting of a metal type, a ceramic type, a graphite type and equivalents thereof. Also, a casting may be performed using gravity casting method, continuous casting method and equivalents thereof. However, the mold type and the casting method are not limited to the above.

In cooling operation S15, the mold is cooled down to a room temperature, and a metal alloy (e.g., metal alloy ingot) is picked out of the mold.

Here, the metal alloy manufactured through the above-described method includes a plurality of metal grains having grain boundaries therebetween, and an intermetallic compound (i.e., Al₂Sc, AlSc or Al₃Sc) existing at the grain boundaries which are not inside but outside the metal grains.

As such, according to an exemplary embodiment, a magnesium mother alloy (Sc-containing magnesium or Sc-containing magnesium-aluminum) is added into a metal melt aluminum alloy), thus making it possible to solve several problems occurring when scandium oxide is directly put into the metal melt. For example, the direct addition of scandium oxide (Sc₂O₃) into aluminum causes the quality of an alloy to be deteriorated due to oxides, however, the addition of Sc-containing magnesium or Sc-containing magnesium-aluminum into aluminum according to an embodiment enables the aluminum alloy to be manufactured at low cost while not deteriorating the quality (hardness, corrosion resistance, weldability, etc.) of an alloy.

Table 3 below shows experimental data for strength of an aluminum alloy manufactured through the above-described method.

**[Table 3]**

| | | |
|---|---|---|
| Strength of 7000-series Al alloy | Including Sc | 650-700MPa |
| | Not including Sc | 550-600MPa |
| Strength of 5000-series Al alloy | Including Sc | 450-500MPa |
| | Not including Sc | 350-400MPa |

As shown in Table 3, it can be understood that the strength increases up to about 650-700 MPa from about 550-600 MPa when magnesium or magnesium-aluminum, into which Sc has been already added, is added into 7000-series Al alloy through the above-described method.

It can be also understood from Table 3 that the strength increases up to about 450-500 MPa from about 350-400 MPa when magnesium or magnesium-aluminum, into which Sc has been already added, is added into 5000-series Al alloy through the above-described method.

As such, in a metal alloy and a method thereof according to the embodiments, a magnesium mother alloy containing Sc is added into a metal alloy such as a magnesium alloy or an aluminum alloy, and thus the metal alloy is manufactured at low cost. Furthermore, alloy properties of the metal alloy, e.g., hardness, corrosion resistance and weldability, are not deteriorated.

In addition, according to the embodiments, the magnesium mother alloy is manufactured in such a form that Sc is dissolved in metal grains, or Sc is crystallized at grain boundaries, which makes it possible to easily manufacture a metal alloy suitable for use or purpose. For example, when a metal alloy where Sc is dissolved is required, a magnesium mother alloy where Sc is dissolved in the metal grains may be used. Also, when a metal alloy where Sc is crystallized is required, a magnesium mother alloy where Sc is crystallized at the grain boundaries may be used. Of course, a metal alloy may be manufactured by adding both of the magnesium mother alloy where Sc is dissolved in metal grains and the magnesium mother alloy where Sc is crystallized at the grain boundaries.

As described above, according to foregoing embodiments, oxidation and ignition properties of a magnesium mother alloy are enhanced by adding scandium oxide into the magnesium mother alloy. Also, a metal alloy can be manufactured at low cost because the magnesium mother alloy containing scandium is added into a metal alloy such as a magnesium alloy and an aluminum alloy. In this case, alloy properties, e.g., hardness, corrosion resistance, and weldability, of the metal alloy are not deteriorated.

Moreover, it is possible to manufacture a metal alloy suitable for use and purpose by preparing two types of mother alloys of which one is a magnesium mother alloy containing scandium dissolved in grains, and the other is a magnesium mother alloy where scandium is crystallized. For example, when a metal alloy where Sc is dissolved is required, a magnesium mother alloy where Sc is dissolved in the metal grains may be used. Also, when a metal alloy where Sc is crystallized is required, a magnesium mother alloy where Sc is crystallized at the grain boundaries may be used. Of course, a metal alloy may be manufactured by adding both of the magnesium mother alloy where Sc is dissolved in metal grains and the magnesium mother alloy where Sc is crystallized at the grain boundaries. Accordingly, according to the embodiments, it is possible to manufacture metal alloys suitable for use and purpose through various methods.

## Claims

1. A method of manufacturing a magnesium mother alloy having a scandium (Sc) for fabricating aluminum, the method comprising:
forming a magnesium melt by putting magnesium into a crucible and melting the magnesium at a temperature ranging from about 600 to about 800 °C;
adding powdered scandium oxide (Sc₂O₃) into the magnesium melt;
stirring the magnesium melt for about 1 to about 400 minutes;
pouring the magnesium melt into a mold having a temperature ranging from a room temperature to about 400 °C and casting the magnesium melt; and
cooling the cast magnesium.

2. The method as claimed in claim 1, wherein, in the forming of the magnesium melt, the magnesium is pure magnesium or magnesium-aluminum.

3. The method as claimed in claim 1 or 2, wherein an added amount of the scandium oxide is about 0.0001 to about 30 parts by weight based on 100 parts by weight of pure magnesium or magnesium-aluminum.

4. A method of manufacturing an aluminum alloy, the method comprising:
forming an aluminum melt;
adding a magnesium mother alloy containing dissolved scandium or scandium compound and produced in accordance with one of claims 1 to 3 into the aluminum melt;
stirring the aluminum melt for about 1 to about 400 minutes;
pouring the aluminum melt into a mold having a temperature ranging from a room temperature to about 400°C and casting the aluminum melt; and
cooling the cast aluminum.

5. The method as claimed in claim 4, wherein an added amount of the magnesium mother alloy containing the scandium is about 0.0001 to about 30 parts by weight based on 100 parts by weight of metal.

6. The method as claimed in claim 4 or 5, wherein the magnesium mother alloy containing the scandium is manufactured by adding about 0.0001 to about 30 parts by weight of the scandium oxide (Sc₂O₃) based on 100 parts by weight of pure magnesium or magnesium-aluminum.

7. The method as claimed in claim 4, wherein the magnesium mother alloy containing the scandium includes an alloy prepared by adding about 0.0001 to about 30 parts by weight of the scandium oxide (Sc₂O₃) based on 100 parts by weight of pure magnesium, and an alloy prepared by adding about 0.0001 to about 30 parts by weight of the scandium oxide (Sc₂O₃) based on 100 parts by weight of magnesium-aluminum.

8. The method as claimed in claim 4, wherein the aluminum melt is formed of one selected from consisting of 1000-series, 2000-series, 3000-series, 4000-series, 5000-series, 6000-series, 7000-series and 8000-series wrought aluminum, and 100-series, 200-series, 300-series, 400-series, 500-series, and 700-series casting aluminum.

## Patentansprüche

1. Herstellungsverfahren einer Scandium (Sc) enthaltenden Magnesium-Vorlegierung zur Produktion von Aluminium, umfassend
- Bildung einer Magnesiumschmelze durch Einsatz von Magnesium in einen Tiegel und Schmelzen des Magnesiums bei einer Temperatur im Bereich von etwa 600 bis etwa 800 °C,
- Zufügen von gepulvertem Scandiumoxid (Sc₂O₃) in die Magnesiumschmelze,
- Rühren der Magnesiumschmelze während etwa 1 bis etwa 400 Minuten,
- Eingießen der Magnesiumschmelze in eine Form mit einer Temperatur im Bereich von Raumtemperatur bis etwa 400 °C und Gießen der Magnesiumschmelze und
- Kühlen des gegossenen Magnesiums.

2. Verfahren nach Anspruch 1, worin bei der Bildung der Magnesiumschmelze das Magnesium reines Magnesium oder Magnesium-Aluminium ist.

3. Verfahren nach Anspruch 1 oder 2, worin die zugesetzte Menge Scandiumoxid etwa 0,0001 bis etwa 30 Gewichtsteile, bezogen auf 100 Gewichtsteile reines Magnesium oder Magnesium-Aluminium, ist.

4. Verfahren zur Herstellung einer Aluminiumlegierung, umfassend
- Bildung einer Aluminiumschmelze,
- Zufügen einer Magnesium-Vorlegierung, welche Scandium oder eine Scandiumverbindung gelöst enthält und nach einem der Ansprüche 1 bis 3 hergestellt wurde, in die Aluminiumschmelze,
- Rühren der Aluminiumschmelze während etwa 1 bis etwa 400 Minuten,
- Eingießen der Aluminiumschmelze in eine Form mit einer Temperatur im Bereich von Raumtemperatur bis etwa 400 °C und Gießen der Aluminiumschmelze und
- Kühlen des gegossenen Aluminiums.

5. Verfahren nach Anspruch 4, worin die zugesetzte Menge der das Scandium enthaltenden Magnesium-Vorlegierung etwa 0,0001 bis etwa 30 Gewichtsteile, bezogen auf 100 Gewichtsteile Metall, ist.

6. Verfahren nach Anspruch 4 oder 5, worin die das Scandium enthaltende Magnesium-Vorlegierung durch Zufügen von etwa 0,0001 bis etwa 30 Gewichtsteilen Scandiumoxid (Sc₂O₃), bezogen auf 100 Gewichtsteile reines Magnesium oder Magnesium-Aluminium, hergestellt wird.

7. Verfahren nach Anspruch 4, worin die das Scandium enthaltende Magnesium-Vorlegierung eine Legierung, die durch Zufügen von etwa 0,0001 bis etwa 30 Gewichtsteilen Scandiumoxid (Sc₂O₃), bezogen auf 100 Gewichtsteile reines Magnesium, hergestellt wurde, und eine Legierung, die durch Zufügen von etwa 0,0001 bis etwa 30 Gewichtsteilen Scandiumoxid (Sc₂O₃), bezogen auf 100
Gewichtsteile Magnesium-Aluminium, hergestellt wurde, umfasst.

8. Verfahren nach Anspruch 4, worin die Aluminiumschmelze gebildet ist aus einer aus der aus Aluminiumknetlegierungen Serie 1000, Serie 2000, Serie 3000, Serie 4000, Serie 5000, Serie 6000, Serie 7000 und Serie 8000 und Aluminiumgusslegierungen Serie 100, Serie 200, Serie 300, Serie 400, Serie 500 und Serie 700 bestehenden Gruppe ausgewählten.

## Revendications

1. Procédé de fabrication d'un alliage mère au magnésium comprenant un scandium (Sc) pour fabriquer d'aluminium, le procédé comprenant les étapes de :
préparer une fonte de magnésium en versant le magnésium dans un creuset et fondant le magnésium à une température dans une plage d'environ 600 à l'environ 800°C;
ajouter à la fonte de magnésium d'oxyde de scandium (Sc₂O₃) pulvérisé;
agiter la fonte de magnésium pendant d'environ 1 à d'environ 400 minutes ;
verser dans une moule ayant une température dans une plage d'une température ambiante à d'environ 400°C la fonte de magnésium et mouler ladite fonte de magnésium ; et
refroidir le magnésium moulé.

2. Procédé selon la revendication 1, dans lequel procédé, à la préparation de la fonte de magnésium, le magnésium est le magnésium pur ou le magnésium-aluminium.

3. Procédé selon les revendications 1 ou 2, dans lequel procédé une quantité ajoutée de l'oxyde de scandium est d'environ 0,0001 à d'environ 30 parties en poids de magnésium pur ou de magnésium-aluminium.

4. Procédé de fabrication d'un alliage d'aluminium, le procédé comprenant les étapes de :
préparer une fonte d'aluminium ;
ajouter à la fonte d'aluminium un alliage mère au magnésium contenant de scandium ou un composé de scandium solutés et produit selon l'une des revendications 1 à 3 ;
agiter la fonte d'aluminium pendant d'environ 1 à d'environ 400 minutes ;
verser la fonte d'aluminium dans une moule ayant une température dans une plage d'une température ambiante à d'environ 400°C, et mouler la fonte d'aluminium ; et
refroidir l'aluminium moulé.

5. Procédé selon la revendication 4, dans lequel une quantité ajoutée de l'alliage mère au magnésium contenant de scandium est d'environ 0,0001 à d'environ 30 parties en poids, par rapport aux 100 parties en poids de métal.

6. Procédé selon les revendications 4 ou 5, dans lequel procédé l'alliage mère au magnésium contenant de scandium est fabriqué en ajoutant d'environ 0,0001 à d'environ 30 parties en poids de l'oxyde de scandium (Sc₂O₃), par rapport aux 100 parties en poids de magnésium pur ou de magnésium-aluminium.

7. Procédé selon la revendication 4, dans lequel procédé l'alliage mère au magnésium contenant le scandium comprend un alliage préparé en ajoutant d'environ 0,0001 à d'environ 30 parties en poids de l'oxyde de scandium (Sc₂O₃), par rapport aux 100 parties en poids de magnésium pur, et un alliage préparé en ajoutant d'environ 0,0001 à d'environ 30 parties en poids de l'oxyde de scandium (Sc₂O₃), par rapport aux 100 parties en poids de magnésium-aluminium.

8. Procédé selon la revendication 4, dans lequel procédé la fonte d'aluminium est préparée de l'aluminium battu choisi parmi la série 1000, la série 2000, la série 3000, la série 4000, la série 5000, la série 6000, la série 7000, la série 8000, et de l'aluminium moulé choisi parmi la série 100, la série 200, la série 300, la série 400, la série 500 et la série 700.
